

# UNITED STATES PATENT OFFICE.

CHARLES J. REED, OF PHILADELPHIA, PENNSYLVANIA.

## ELECTROLYTIC PROCESS.

1,055,652.

Specification of Letters Patent.

Patented Mar. 11, 1913.

No Drawing. Original application filed May 10, 1911, Serial No. 626,148. Divided and this application filed June 3, 1912. Serial No. 701,296.

To all whom it may concern:

Be it known that I, CHARLES J. REED, a citizen of the United States, residing at Philadelphia, county of Philadelphia, and State of Pennsylvania, have invented certain new and useful Improvements in Electrolytic Processes, of which the following is a specification.

My process relates to the electrolytic deposition and recovery of iron from its solution as sulfate.

The electrolytic deposition of the highly magnetic metals, nickel, iron and cobalt, from sulfate solutions with an anode which does not go into solution, like the electrolytic deposition of zinc under the same conditions, is subject to the difficulty that the metal is not easily or efficiently deposited in the presence of free sulfuric acid, and as the percentage of free acid in the solution increases, the deposition of the metal with a given current decreases. This difficulty was overcome in the case of zinc by a process described by Carl Hering in U. S. Letters Patent No. 798,790, granted September 5, 1905.

Iron has the same property as zinc of being unreduced and unaffected in solution as sulfate by contact with metallic lead. I find that an anode of spongy lead may be used to combine with the  $(SO_4)$  of the sulfate of this metal to produce insoluble sulfate of lead and prevent the liberation of free sulfuric acid in the electrolyte. This enables me to electrolytically deposit the metal from its sulfate solution without the inefficiency due to the presence of free sulfuric acid.

In the operation of my process, I prepare a solution of the sulfate of iron and electrolyze it with a cathode of any suitable conducting substance, such as carbon, copper, aluminum or any conducting body on which it is desired to deposit the iron, and an anode of spongy or finely-divided lead, such as is usually employed in the negative plates of a lead accumulator. The sum of the reactions which take place may be represented by the following chemical equation:



This means that the metallic lead combines with the  $SO_4$  of the iron sulfate and the iron is set free in the metallic state, there being no other chemical changes in

the solution. If this operation were allowed to continue, the spongy lead would eventually all or nearly all be converted into lead sulfate. But in practice I find it advisable to allow only about one-third or less of the spongy lead to become sulfated, as is the general practice in the discharge of an accumulator. When this has occurred I remove the anode (replacing it with a fresh one) and place it in a dilute solution of sulfuric acid and pass an electric current through it in the opposite direction, using it as a cathode until the lead sulfate has all or nearly all been reduced to metallic spongy lead and the  $SO_4$  liberated as sulfuric acid. The electrode may then be again used as an anode in the deposition cell and the operation becomes cyclic, the sulfuric acid being a by-product which may be recovered and utilized.

I do not limit myself to the use of any particular substance as a cathode for receiving the deposit of iron, but prefer a sheet of nickel or aluminum.

By the term "anode of spongy lead" as herein used, I do not mean that the entire electrode consists necessarily of spongy lead, but only that it contains spongy lead as chemically-active material. It may, for example, be made up of a conducting framework of hard lead, antimonial lead or other suitable material capable of conducting the electric current and having spongy lead applied to or contained in it, as in the ordinary accumulator plate.

This application is a division of Serial No. 626,148, filed May 10, 1911.

I claim:

1. The process of recovering metallic iron from a solution of its sulfate, which consists in electrolyzing said solution, using an anode of spongy lead, substantially as herein described.

2. The process of depositing metallic iron from its solution as sulfate, which consists in electrolyzing said solution, using an anode of spongy lead, and subsequently regenerating said anode material in a separate receptacle, substantially as herein described.

3. The process of reducing metallic iron from its solution as sulfate, which consists in electrolyzing said solution, using an anode of spongy lead, and electrolytically regenerating said anode material in a sepa-

rate receptacle, substantially as herein set forth.

4. The process of recovering metallic iron from a solution of its sulfate, which consists in electrolyzing said solution, using an anode of spongy lead, electrolytically regenerating said anode material in a separate receptacle, and recovering the sulfuric

acid as a by-product, substantially as herein described.

In testimony whereof I affix my signature in presence of two witnesses:

CHARLES J. REED.

Witnesses:

FRANK A. LEACH,  
J. M. JACKSON.